

(No Model.)

G. H. KNIGHT.  
PENCIL.

No. 588,867.

Patented Aug. 24, 1897.



Witnesses:

Fred R. Proctor  
Karl H. Henning.

Inventor:

Geo. Hy. Knight  
By Knights Bros  
Atlys.

# UNITED STATES PATENT OFFICE.

GEORGE HENRY KNIGHT, OF LYNN, MASSACHUSETTS.

## PENCIL.

SPECIFICATION forming part of Letters Patent No. 588,867, dated August 24, 1897.

Application filed May 7, 1897. Serial No. 635,563. (No model.)

To all whom it may concern:

Be it known that I, GEORGE HENRY KNIGHT, a citizen of the United States, residing at Lynn, in the county of Essex and State of Massachusetts, have invented a new and useful Improvement in Pencils, of which the following is a specification.

My invention is a device for a point-maintaining or self-sharpening pencil or crayon.

10 In this specification "graphite" or "graphite composition" may signify any dry solid used for marking purposes which is obtainable of several grades of hardness.

While applicable to caseless pencils ("crayons") and available with any suitable marking material, my invention is more especially designed for, and is here described as, an improvement in "black lead-pencils," so called, whose "lead" or "filling" is of a graphite 20 composition. My improvement relates wholly to the filling.

My improved filling consists of a slender rod or filament (preferably of graphite or a preparation thereof) which forms the core, center, or nucleus to a surrounding sheath, body, or coating of like but softer material, or to two or more such successively softer concentric layers or coatings. Being applied in a viscous condition said coatings on solidifying unite with the core and with one another to form the closely-adherent mass of soft exterior and relatively hard central portion which constitutes my composite filling.

My invention is illustrated to a greatly-enlarged scale in the accompanying drawings.

Figure I represents a "core" or "center." Fig. II represents a completed filling of the simplest ("binary") form. Fig. III shows the finished pencil, and Fig. IV the same pointed for use. Fig. V represents a "multiplex" filling, and Fig. VI the same incased. Figs. VII and VIII are cross-sections of the pencils shown at Figs. IV and VI. Figs. IX, X, and XI show a modified construction to a greatly-enlarged scale.

The simplest (binary) form of my filling is seen in Figs. II, III, IV, and VII, in which a core, center, or nucleus *a* is shown combined with a closely-adherent encircling and sup-

porting shell, sleeve, or coating *b*, of softer graphite, which when solidified forms with said core *a* a composite but solid rod. Instead of being used in this form directly as a filling the rod *a b* may receive an added coating *c*, Figs. V, VI, and VIII, (or a series of such 55 coatings,) so as to form a multiplex filling. No coating is applied until solidification of the interior portions, and for each addition a softer marking graphite is selected and is applied in a viscous condition. Such application may be made by immersion of the core or solid nucleus in the viscous or semiliquid coating material. Inclosure may take place in the stock or casing *d* before the peripheral or last applied coating of the core has fully 60 solidified. For manufacture of fillings with very slender cores grooved shell partings *b<sup>I</sup>x b<sup>II</sup>*, (shown in Fig. IX,) or *b<sup>III</sup>x b<sup>IV</sup>*, (shown in Fig. X,) or *b<sup>V</sup>x b<sup>VI</sup>*, (shown in Fig. XI,) being coated with viscous graphite, the core while 65 plastic is placed in groove *x* and the parts closed together. A still different mode of manufacture may consist in treating the peripheral portions with glycerin or other softening agent, leaving the hard central portion 70 intact. Cutting into pencil lengths may take place at any convenient stage of the process.

I claim herein as new and of my invention—

1. As a new and useful article of manufacture; the point-maintaining pencil comprising a central rod or core of hard marking material and one or more concentric sleeves of successively softer marking material in which the rod or core is incased; substantially as set forth.

85 2. A pencil-filling which consists of the combination of a central graphite core *a*, with an inclosing shell or coating *b*, of like but softer material; for the purpose set forth.

3. A pencil-filling composed of the combination of a graphite center *a*, and the closely-adherent supporting-sleeve *b*, of softer graphite composition; substantially as described and for the purpose set forth.

90 4. In the described combination; a central core *a*, of marking material and one or more tubular closely-adhering coatings *b, c*, of like, but successively softer material, as set forth.

5. The combination with a suitable casing; of the composite filling composed of a graphite center within one or more adherent tubes of a softer graphite composition.
- 5 6. The described combination with a casing *d*, of a filling which consists of the graphite core or center *a*, and a series of adherent, tu-

bular layers or coatings *b*, *c*, of successively softer graphite compositions; for the purpose explained.

GEORGE HENRY KNIGHT.

Witnesses:

M. E. KNIGHT,  
CHARLES W. GEER.